

Oct. 9, 1923.

1,469,817

I. RENNERFELT

METHOD OF ELECTRICALLY MELTING METALS AND IN AN ELECTRIC FURNACE

Filed June 16, 1921

*Fig. 1.*



*Fig. 3.*



*Fig. 2.*



Witnesses:

*John Holmgren  
Per Klemm*

inventor:

*Isaac Rennerfelt*

## UNITED STATES PATENT OFFICE.

IVAR RENNERFELT, OF DJURSHOLM, SWEDEN.

## METHOD OF ELECTRICALLY MELTING METALS AND IN AN ELECTRIC FURNACE.

Application filed June 16, 1921. Serial No. 478,095.

*To all whom it may concern:*

Be it known that I, IVAR RENNERFELT, a citizen of the Kingdom of Sweden, and resident of Djursholm, in the county of Stockholm Lan and Kingdom of Sweden, have invented a certain new and useful Improvement 5 in Methods of Electrically Melting Metals and in an Electric Furnace (for which I filed application in Sweden, Oct. 22, 1919), of which the following is a specification.

My invention relates to a certain improved method of electrically melting metals and especially iron and steel. It 15 relates also to an electric furnace, which is well adapted to be used in connection with the method referred to. The objects of my invention are, first, to disclose a method for melting economically a large quantity 20 of metal with a comparatively small power, the method being especially characterized by this, that the melting time is very long, in most cases preferably close to 24 hours, second, to disclose how an electric furnace 25 should be built to permit the accumulation of a considerable quantity of electric energy without an excessive loss of kilowatthours and to facilitate storing a considerable 30 quantity of liquid metal, for instance steel or pigiron, discharging it in a very short time; and, third, to provide means, which will make it possible to introduce electric 35 melting on a large scale in the foundries making ordinary gray or malleable iron castings.

The nature of the work in such foundries requires that a big quantity of liquid iron shall be available at a certain time, generally 40 in the afternoon. Usually the iron is melted in one or more cupola furnaces or open hearths, delivering the iron at a certain practically constant rate of melting, the metal being taken to the moulds practically 45 without stopping. If the number of cupolas is insufficient, or if their melting capacity is rather small, the time required for pouring the iron into the moulds will be quite 50 considerable, causing a very considerable loss of time, which could with advantage be used for moulding work. The present 55 foundry practice, however, prevents this saving of time, because it is practically impossible to carry on any moulding work after the pouring of the iron has once

started filling the foundry with smoke and disturbances of many kinds. It is, furthermore, well known, that generally no pouring is possible during the regular time of moulding, and therefore the iron must be melted as quickly as possible after the 60 moulding work is done.

A medium-sized foundry may use some 50 tons of iron daily. To melt this electrically would require about 20,000 kwhrs. For melting the iron in 5 hours not less than 65 4,000 kw. would have to be supplied. This is hardly possible, as the cost of installation would be rather high and also the cost of the energy on account of the very bad load factor. If, however, the melting is going on 70 day and night at a constant rate the power required would be only about 1,000 kw., which would be much cheaper to provide. To lessen still more the electric power required it is possible to combine electric melting with cupola melting, keeping the electric melting going during the night, obtaining a specially cheap rate for the energy, melting in the cupola during the day and storing 75 the cupola iron in the electric accumulating 80 and melting furnace. It is of course possible and generally also necessary to supply a certain amount of power to the electric furnace to keep the iron hot, and, if desired, to overheat it. The combination of the 85 cupola with the electric furnace is especially valuable in places, where the coke is cheap but the electric energy expensive.

It is obvious that the iron will be greatly improved by being accumulated and heated 90 to a very high temperature in a preferably basic electric furnace. Not only will the amount of sulphur decrease, but the iron will also contain less gases and slag.

It is also possible to soften a hard iron 95 and to make corrections regarding the amount of manganese, silicon and other elements.

If melting simultaneously in the electric furnace and in the cupola the latter may be 100 comparatively small, being kept at maximum melting output all the time, which will increase the efficiency and lessen the amount of coke as no cooling off of the cupola lining will take place from one day to the 105 other, as is now customary.

It is obvious that it also is a considerable improvement upon the general foundry

practice to accumulate a large quantity of high grade iron, making it possible to cast very heavy pieces with great convenience.

The method disclosed in my invention 5 means also another improvement upon the foundry practice by making it possible to postpone the pouring a certain time in the afternoon, if the moulding work should so require. It is also possible to tap the furnace for instance in the morning if required.

In order to successfully use the method of melting according to my invention the furnace should be carefully built along certain 15 lines. The insulation against loss of heat must be most excellent. Consequently the geometrical shape best suited to all purposes would be that of a cylinder resting on bearings, permitting it to be rotated for 20 discharging as usual with mixers.

The charging openings should be quite few and of small size as no big objects, but only liquid iron or common pigiron bars will as a rule be charged into the furnace. 25 The charging openings may conveniently be placed one in each end of the cylinder. The discharging openings should preferably be made as ordinary tapholes with or without means for closing, located in the ends of 30 the hearth and preferably also one or more in the cylindrical wall. It is desirable to use several tapholes located at different places so as to permit several men to get iron in their handladles simultaneously, 35 preventing the usual, undesirable crowding of moulders at the single taphole of the cupola or open hearth. The tapholes should be located on the same level and preferably above the highest level of a full charge of 40 iron in the furnace. By having the tapholes above the level of charge it will be possible to keep the holes clear from freezing and in good shape.

To withdraw the liquid iron through tapholes at the bottom of a furnace of the mixer type is practically impossible, because 45 of the considerable head of the iron above the hole, which would cause a high tapping velocity of the iron on flowing out, causing 50 also serious difficulties, if it should become necessary to close the taphole, after it has been opened. The end tapholes should be located close to the inside cylindrical wall to 55 make it possible to discharge the whole charge through said holes.

To facilitate withdrawal of slag when necessary the charging openings in the ends of the hearth may be extended sideways so far as to make the charge overflow to a certain degree, when the furnace is being rotated, in this way causing the slag to be discharged.

To supply the electric energy into the furnace several electrodes may be arranged 60 to project into the hearth from above. If

using only such electrodes, which are practically vertical, when the furnace is in its normal melting position, the heat will be generated in the usual way by means of arcs in contact with the charge.

70

It is possible also to use electrodes entering through the sides at a certain convenient angle to the horizontal plane cooperating with each other or with vertical electrodes to form arcs burning above the surface of the 75 iron.

The furnace may be rotated considerably to one or both sides in order to cause movements in the bath for mixing it thoroughly. By rotating the furnace new parts of the 80 lining will be brought in contact with the bath getting cooled by this, if hotter than the iron. Rotating the furnace in this way requires closing the discharge openings temporarily by suitable means or locating all 85 the holes high enough to permit a considerable rotation without the contents flowing out.

When rotating the furnace for mixing or discharging the iron it may be practical to 90 withdraw the electrodes from the interior keeping them suspended in the air above the furnace, as is well known in the electric furnace practice.

Under certain circumstances it may be desirable when tapping the metal to make the furnace roll on horizontal beds instead of 95 rotating it as previously described, but the last method will probably be used more often than the former.

On the accompanying drawing Fig. 1 shows a vertical section at  $x-x$  in Fig. 2, which is a top view of a furnace according to the present invention, provided with three vertical electrodes. Fig. 3 is a vertical section of a furnace having two or more sets of electrodes, each set consisting of two 105 adjustable electrodes entering from opposite sides at about  $45^{\circ}$  angle from the horizontal plane. A third vertical electrode may 110 be used as indicated by dotted lines.

On the drawing a cylindrical melting hearth is indicated by 1, roller bearings supporting the hearth by 2 and a charge of 115 liquid metal by 3. Electric arcs are indicated by 4 and electrodes 5 project vertically into the hearth and other electrodes 6 may project into the hearth at a considerable angle to the vertical line. In the end wall of the furnace tapholes 7 are provided 120 close to the inside cylindrical wall at convenient places on one or both sides of the hearth. To facilitate charging of cold or liquid metal openings 9 are provided in the end wall, closed by tightly fitting doors 10.

The openings 9 may be extended wide enough to one or both sides to cause the lower corner to dip underneath the level of the charge so as to cause the slag or the charge itself to overflow when rotating the 130

hearth in the proper way. The tapholes 7 and 8 may, if desired, be provided with snugly fitting stoppers to be handled from the outside and permitting the metal to be withdrawn from the hearth in the same manner as steel is tapped from a ladle provided with means for tapping through the bottom.

I do not wish to limit myself to the exact shape of the furnaces illustrated on the drawing as several modified forms are possible without departing from the scope of my invention. It would for instance be possible to provide also bottom contacts as indicated by 11 for supplying electric energy to the charge without using arcs for generating the heat.

Having now fully described my invention I claim and desire to secure by Letters Patent of the United States of America.

1. The method of melting a metal which consists in providing a carefully insulated electric furnace charging it gradually with metal at a certain rate extending over nearly twenty-four hours time and causing the metal to melt by supplying electric power at a rate, which is sufficient to cover the loss of heat from the furnace and to furnish the amount of heat required for melting slowly the quantity of metal intended to be discharged about once every twenty-four hours.

2. The method of melting a metal, which consists in providing a carefully insulated electric furnace and a cupola furnace charging the electric furnace gradually with metal at a certain rate extending over nearly

twenty-four hours time, taking the metal in liquid state from the cupola, keeping this melting continuously for nearly twenty-four hours and supplying sufficient power to keep the metal hot in the electric furnace, discharging it about once every twenty-four hours.

3. The method of melting a metal which consists in providing a carefully insulated electric furnace and a cupola furnace charging the electric furnace gradually with cold metal during the night and with liquid metal from the cupola at daytime supplying sufficient power to melt the cold charge in the electric furnace and to keep the liquid bath hot at daytime, discharging it in the afternoon.

4. In an electric furnace the combination of a preferably cylindrical melting hearth with electrodes projecting through the cylindrical side, means for lowering one side of the furnace and simultaneously lifting the opposite side, openings in the endwalls close to the inside surface of the cylindrical wall and a charging opening in the end wall, located so as to cause a layer of slag on top of a charge of metal to overflow when lowering one side of the hearth sufficiently.

Signed at Stockholm in the county of Stockholm Lan and State of Sweden this 21st day of May A. D. 1921.

IVAR RENNERFELT.

Witnesses:

ENEZ IVERSON,  
WIEMER C. ERIKSON.